

3,321,400

**LUBRICANT CONTAINING PHOSPHOSUL-FURIZED HYDROCARBON DERIVATIVE**

Alexander von Hoyningen-Huene, Buchholz i. d. Nordheide, and Siegfried Slabon, Hamburg-Neugraben, Germany, assignors to Esso Research and Engineering Company, a corporation of Delaware  
 No Drawing. Filed May 25, 1965, Ser. No. 458,755  
 Claims priority, application Germany, July 4, 1964,  
 E 27,339

6 Claims. (Cl. 252—46.7)

Lubricants having as many-sided properties as possible are of constantly increasing significance in view of plant simplification and rationalisation. If a lubricant can simultaneously fulfill several lubricating functions, it is to be preferred, from the operational point of view, to the use of several lubricants of specific effect. Consequently, substituting one polyfunctional product for several lubricants constitutes a step forward in the art.

Lubricants having polyfunctional properties that can find a wide field of application are e.g. those which can simultaneously be used in engines, gears, and hydraulic systems. The specific properties required for these fields of use are in part widely different. A lubricant that is capable of satisfying the various demands has to be adjusted very closely to the various functions it has to fulfill. Below is a list of the various properties of a lubricant (apart from mere lubrication) that are significant for the various fields of use.

| Field of application                                   | Properties demanded                                                                                                                                                                                                                                                                                                                                                                                                                                                                                                                                                                                                                                           |
|--------------------------------------------------------|---------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| A. Engine                                              | <ul style="list-style-type: none"> <li>(a) Cleaning effect (detergent-dispersant).</li> <li>(b) Neutralizing property towards acid combustion products.</li> <li>(c) Oxidation (age) resistance.</li> <li>(d) Load absorbing power.</li> <li>(e) Corrosion protection.</li> <li>(f) Indifference to sealing material.</li> <li>(g) Low viscosity.</li> <li>(h) Good viscosity-temperature behaviour.</li> <li>(i) Good low-temperature performance.</li> <li>(j) Heat resistance.</li> <li>(k) Dispersing ability.</li> <li>(l) Age resistance.</li> <li>(m) Corrosion resistance.</li> <li>(n) In certain cases also extreme pressure properties.</li> </ul> |
| B. Gears (gear box, rear axle drive gears).            |                                                                                                                                                                                                                                                                                                                                                                                                                                                                                                                                                                                                                                                               |
| C. Hydraulic or hydraulic-mechanic power transmission. |                                                                                                                                                                                                                                                                                                                                                                                                                                                                                                                                                                                                                                                               |

As is shown in the list, there are in part great differences in the properties.

Thin motor oils, e.g. can be employed in highly loaded gears under certain conditions and mostly not at all. In hydraulic systems they may occasionally be used, but in critical cases their properties do not suffice.

On the other hand the use of gear oils or typical hydraulic oils is out of the question for engine purposes due to their lack of detergent and neutralizing effect.

Thus any lubricant equally well suited for the application fields A, B, and C has to contain an additive or additive combination which is capable of fulfilling the demands involved.

It has now been found that a lubricant additive that greatly satisfies those demands is obtained by reacting polybutenes that have been treated with phosphorous (V) sulfide with a long-chained monohydric alcohol, preferably an unsaturated alcohol, for example, oleyl alcohol, and if desired reacting the resulting reaction product further with a polyamine. The term "polybutenes" covers all the polymers of butenes, also of isobutylene.

The use of  $P_2S_5$ -treated polybutenes in conjunction with alkaline earth hydroxides or in combination with alkaline earth phenolates as lubricant additives has been described in numerous patents.

However, because of excessive corrosion it is impossible to use that product by itself although it is dispersing and extreme pressure effective. But in the reaction of  $P_2S_5$ -treated polybutenes (molecular weight 500 to 2000) with alcohols, products are obtained which in comparison with the starting material show improvements regarding the following properties:

- (1) Corrosion behavior
- (2) Acidity (greatly reduced)
- (3) Dispersing ability
- (4) Heat resistance

In addition, a minor improvement in viscosity-temperature behavior is achieved in the oils to which these products are added.

It was found that the most favourable alcohol for the reaction of the  $P_2S_5$ -treated polybutene is oleyl alcohol. Tests have shown that this alcohol is preferable to the saturated higher alcohols.

If this reaction product is reacted in a second process step with an amine (polyamine), further improvements in the corrosion behavior, acidity and dispersing ability are obtained, whereas heat resistance and extreme pressure behavior are not negatively affected. The corrosion behavior is even improved thereby to such a degree that the product can indeed be considered a corrosion protection. The polyamine employed was dipropylene triamine, however, tetra-ethylene pentamine can also be used.

The lubricant of the invention for engines, gears, hydraulic-mechanic or hydraulic systems on a lubricating oil base is characterized by containing, in proportions of from 1 to 20, preferably from 3 to 5 wt. percent, (a) the product of a reaction of a polybutene treated with phosphorous (V) sulfide and having a molecular weight of 500 to 2000 reacted with a monohydric alcohol, preferably having from 12 to 22 carbon atoms per molecular or (b) reaction product of (a) reacted with a polyamine.

The lubricating oils employed are preferably mineral lubricating oils, particularly paraffin base solvent raffinates.

In addition, the lubricants of the invention can contain, as lubricant additives known per se, metal sulfonates, metal alkyl phenolates, metal alkyl salicylates, metal salts of reaction products of phosphorous (V) sulfide and polybutene or metal amino alkyl phenolates as ash containing detergents in concentrations of from 0.5 to 20.0 wt. percent, metal dialkyl dithiophosphates in concentrations of from 0.1 to 3 wt. percent, extreme pressure additives on the basis of sulfur, chlorine and/or phosphorous in concentrations of from 0.5 to 10 wt. percent, metal deactivators in concentrations of from 0.01 to 1 wt. percent, and/or alkyl succinic acid imides, copolymers of methacrylic acid and amines, or copolymers of vinyl acetate, fumaric acid esters and maleic acid as dispersers in proportions of from 0.5 to 5 wt. percent.

The preparation of the lubricating oil additives to be employed according to the invention, can be carried out as follows:

A polybutene reacted with phosphorus (V) sulfide (molecular weight 500 to 2000) having a phosphorus content of from 2 to 8 wt. percent and a sulfur content of from 4 to 16 wt. percent is reacted for 1 hour at 130 to 200° C. with from 15 to 50 wt. percent, preferably 25 wt. percent, based on the phosphosulfurized polybutene of, a monovalent, high molecular weight, preferably unsaturated fatty alcohol.

The resulting reaction product can if desired be reacted in a second process step for half an hour at 80 to 150° C. with from 1 to 20 wt. percent polyamine (based on the reaction product obtained in the first step).

**3**  
*Example 1*

A lubricating oil additive according to the invention is prepared as follows:

75 g. of a reaction product of  $P_2S_5$  and polybutene (average molecular weight about 700, phosphorus content 85 wt. percent, sulfur content 6.4 wt. percent) are stirred for 1 hour at 175° C. with 25 g. technical oleyl alcohol. In the reaction hydrogen sulfide escapes and the alcohol concentration recedes, which is noted from a reduction of the OH-concentration in the ultrared spectrum. After 10 hours the reaction is finished, which is seen from the complete disappearance of the OH-group in the ultrared spectrum.

When the product has been cooled to 130° C., 3 wt. percent dipropylene triamine is added and the mixture is stirred for 30 minutes. The conclusion of the reaction is apparent from the complete disappearance of the  $NH_2$ -group in the ultrared spectrum. The reaction is about 15 00%.

The reaction product is a dark red viscous liquid that requires no further purification. It is miscible with mineral oils as well as with aliphatic, aromatic and naphthenic hydrocarbons in any proportion.

A corrosion test is conducted as follows:

Batches of 95 wt. percent each of a mineral lubricating oil (viscosity about 50 cs. at 50° C.) are mixed with 3 wt. percent of each of the following additives:

- (1) polybutene treated with phosphorus (V) sulfide (molecular weight 700),
- (2) reaction product of (1) with oleyl alcohol,
- (3) reaction product of (2) with dipropylene triamine.

Each bath of 98 ml. of the oil mixed with the respective additive is stirred with 2 ml. water. A copper strip and a bearing segment (ball bearing basin) are placed in each of the mixtures and left therein for 48 hours at 100° C. The results are as follows:

| Oil mixture | Findings              |                           |
|-------------|-----------------------|---------------------------|
|             | Steel                 | Copper                    |
| (1) -----   | Very greatly corroded |                           |
| (2) -----   | Light rust            | Moderate sulfide coating. |
| (3) -----   | No rust               | Dark brown discolouring.  |

Also when higher concentrations are employed, the additives according to the invention supply satisfactory results in this respect.

*Example 2*

97 wt. percent of a mineral oil SAE is blended with 3 wt. percent of the above described reaction product of  $P_2S_5$  treated polybutene, oleyl alcohol and dipropylene triamine.

This lubricating oil mixture is tested under full load in a one-cylinder diesel engine for 50 hours, the fuel containing 1 wt. percent sulfur. A comparison test is conducted with a commercial HD oil which comprises an ash-containing detergent. The results are as follows:

Total piston performance  
(100 max.)

Lubricating oil: 88  
Lubricating oil according to invention ----- 88  
Comparison oil ----- 89

The comparison shows that the cleansing effect in the engine is definitely favourable for an ash-free product.

*Example 3*

In combination with ash-containing detergents the above described additive according to the invention, in a 50-hour test in a 4-cylinder diesel engine, shows results similar to those of the conventional ash-free dispersing agents, which, however, contrary to the inventive additive, have a dispersant effect only and no other effect to

**4**

improve the lubricating oil. The results of these tests are as follows:

| 5 | Composition                                                                                    | Piston performance (100=max.) |
|---|------------------------------------------------------------------------------------------------|-------------------------------|
|   | Mineral lubricating oil SAE 20+6% ash-containing detergent+1.3% commercial ash-free dispersant | 96                            |
|   | Mineral lubricating oil SAE 20+6% ash-containing detergent+2% additive according to invention  | 94.5                          |

*Example 4*

The dispersant effect, which is of great significance for motor and hydraulic operation, is tested in the following manner:

0.1 g. standard black is stirred into a solution of 1.0 g. lubricating oil additive in 100 ml. normal gasoline. The mixture is transferred to a 100 ml. measuring cylinder and checked for possible sedimentation in the course of 14 days.

| 20 | Mixture                                                                     | Findings after 14 days                                                                |
|----|-----------------------------------------------------------------------------|---------------------------------------------------------------------------------------|
|    | (a) Gasoline and black                                                      | Immediate sedimentation.                                                              |
| 25 | (b) (a)+1 g. $P_2S_5$ -treated polybutene                                   | Complete sedimentation.                                                               |
|    | (c) (a)+1 g. additive according to invention                                | Slight sedimentation major proportion dispersed.                                      |
|    | (d) (a)+1 g. dispersing agent on polymethacrylate amino base                | The same.                                                                             |
| 30 | (e) (a)+1 g. copolymer of vinyl acetate, fumaric acid ester and maleic acid | Slightly increased sedimentation, but still sufficient proportion of dispersed black. |

Even when it was left standing for several months, the additive according to the invention still showed excellent dispersant capacity, thus ensuring flawless sludge-dispersing behaviour in the engine.

*Example 5*

The extreme pressure properties of the lubricants according to the invention are tested in the Four Ball Tester, on the FZG gear test stand, and in a Mercedes rear axle.

40 The above described additive according to the invention is dissolved in a mineral oil SAE 30 in a concentration of 6 wt. percent. The oils are then tested according to the above indicated methods, the results being as follows:

| 45 | Device                 | Result                                                                                                           |
|----|------------------------|------------------------------------------------------------------------------------------------------------------|
|    | Four Ball Tester ----- | Wear 0.33 m. (unalloyed oil 0.6 mm.). Wear data: 260 KG (unalloyed oil 140 kg.).                                 |
| 50 | FZG Test -----         | No switch-over to high wear level, minor chambers in the 12 load steps (comparable to hypoid oils).              |
|    | Rear axle -----        | High wear in 9th step (54.5 kg). Normal behaviour up to 9th load stop (one step lower than typical hypoid oils). |

55 The above values show that the extreme pressure properties of these oils almost correspond to those of a hypoid gear oil that satisfies the highest demands. This is of special significance because the conventional dispersants and detergents are known to have no extreme pressure properties.

*Example 6*

The behaviour towards sealing material is determined by tests in which a "simmering-material" of L. Freudenberg, Weinheim, is kept in contact with the oil base and the oil base containing the inventive additive for 100 hours at 130° C. The results are as follows:

| 70 | Lubricating Oil                                           | Change in Shore-hardness, units | Change in volume, percent |
|----|-----------------------------------------------------------|---------------------------------|---------------------------|
|    | Mineral oil SAE 30                                        | -1                              | +1.6                      |
|    | 95% mineral oil SAE 30-5% additive according to invention | -1                              | +2.3                      |

These values are extraordinarily favourable, since effective extreme pressure additives are known to cause hardening up to 5 Shore units.

*Example 7*

Also the heat resistance of the additive according to the invention as well as of the lubricating oils prepared therewith is very high. This is shown by the following test results:

| Lubricating oil additive                                       | Findings after 7 hours at 175° C.                           |
|----------------------------------------------------------------|-------------------------------------------------------------|
| Additive according to invention                                | No change.                                                  |
| Commercial gear oil additive on phosphorus sulfur base.        | Over 2% insoluble parts.                                    |
| Commercial zinc dialkyl dithiophosphate.                       | Spontaneous decomposition.                                  |
| Lubricating oil mixture                                        | Findings after 100 hours at 130° C.                         |
| 5% additive according to invention in mineral oil SAE 30.      | No change.                                                  |
| 5% commercial extreme pressure additive in mineral oil SAE 30. | Oil-insoluble sediments.                                    |
| 2% zinc dialkyl dithiophosphate in mineral oil SAE 30.         | Decomposition products of the zinc dialkyl dithiophosphate. |

*Example 8*

The good stability of the lubricants according to the invention in prolonged contact with hot metal parts is shown by the following comparative tests, wherein the lubricating oil that contains the additive is pumped in recycle over a tin plate strip heated to 275° C. for 5 hours ("BASF Strip Test").

| Lubricating oil mixture                                                       | Findings of tin plate strip | Weight of the sediment products the tin plate, mg. |
|-------------------------------------------------------------------------------|-----------------------------|----------------------------------------------------|
| 3% additive according to invention, 97% mineral oil SAE 10.                   | Tarnishing colours          | 7                                                  |
| 3% commercial ash-free dispersant, 97% mineral oil SAE 10.                    | Brownish sediment           | 10                                                 |
| 3% P <sub>2</sub> S <sub>3</sub> -treated polybutene, 97% mineral oil SAE 10. | Brownish-black sediment.    | 30                                                 |

What is claimed is:

1. A lubricating oil composition comprising a major

proportion of a mineral lubricating oil to which has been added in the range of from 1 to 20 wt. percent of a poly functional additive obtained by first treating polybutene of molecular weight in the range of 500 to 2000 with P<sub>2</sub>S

- 5 to prepare phosphosulfurized polybutene of phosphorus content in the range of 2 to 8 wt. percent and sulfur content in the range of 4 to 16 wt. percent, thereafter reacting the phosphosulfurized polybutene with from 15 to 50 wt. percent, based on said phosphosulfurized polybutene, of a monovalent unsaturated fatty alcohol of from 12 to 22 carbon atoms, and subsequently treating the product of the last recited reaction with from 1 to 20 wt. percent (based on said last recited product) of an alkylene polyamine having from 3 to 5 amino groups, said polyfunctional additive imparting to said composition corrosion inhibiting, detergent, dispersant, and extreme pressure properties.

2. A lubricating oil composition as defined by claim 1 wherein said reaction with said unsaturated fatty alcohol is conducted at a temperature in the range of from about 130 to 200° C. and wherein said reaction with said polyamine is conducted at a temperature in the range of from about 80 to 150° C.

3. A lubricating oil composition as defined by claim 1 wherein said unsaturated fatty alcohol is oleyl alcohol.

4. A lubricating oil composition as defined by claim 1 wherein said alkylene polyamine is dipropylene triamine.

5. A lubricating oil composition as defined by claim 1 wherein said alkylene polyamine is tetraethylene pentamine.

6. A lubricating oil composition as defined by claim 1 wherein said polyfunctional additive is present in a concentration in the range of about 3 to 5 wt. percent.

**References Cited by the Examiner**

**UNITED STATES PATENTS**

|           |         |               |       |          |
|-----------|---------|---------------|-------|----------|
| 2,356,073 | 8/1944  | May           | ----- | 252—48.4 |
| 2,392,252 | 1/1946  | May           | ----- | 252—32.7 |
| 2,619,462 | 11/1952 | Beare         | ----- | 252—46.7 |
| 2,809,934 | 10/1957 | Alford et al. | ----- | 252—32.7 |
| 2,849,398 | 8/1958  | Moody et al.  | ----- | 252—32.7 |

DANIEL E. WYMAN, *Primary Examiner.*

45 L. G. XIARHOS, W. H. CANNON,

*Assistant Examiners.*